

March 1, 1955

W. L. FINLAY ET AL

2,703,278

TITANIUM-ALUMINUM ALLOYS

Filed April 23, 1954



Fig. 1



Fig. 2 *Ward, Heald, Charlton, Dume & McElhaney*  
ATTORNEYS

INVENTORS  
WALTER L. FINLAY  
BRUCE W. CONSER  
ROBERT I. JAFFEE

1

2,703,278

## TITANIUM-ALUMINUM ALLOYS

Walter L. Finlay, Beaver, Pa., and Bruce W. Gonser, Columbus, and Robert L. Jaffee, Worthington, Ohio, assignors, by direct and mesne assignments, to Rem-Cru Titanium, Inc., Midland, Pa., a corporation of Pennsylvania.

Application April 23, 1954, Serial No. 425,134.

11 Claims. (Cl. 75—175.5)

This invention pertains to binary alloys of titanium and aluminum and also to ternary and higher alloys of titanium and aluminum containing one or more of the interstitial elements carbon, oxygen and nitrogen.

This application is a continuation-in-part of our co-pending application Serial No. 157,639, filed April 22, 1950; Serial No. 179,322, filed August 14, 1950; and Serial No. 210,439, filed February 10, 1951, now abandoned, which are in turn continuations-in-part of our now abandoned applications Serial No. 66,838, filed December 22, 1948, and Serial No. 95,152, filed May 24, 1949.

Substantially pure titanium can be produced by the so-called "iodide" process described in Patent No. 1,671,213 to Van Arkel, but the process is slow and expensive. Titanium is accordingly commercially produced at the present time principally by the magnesium reduction of titanium tetrachloride, in accordance with the process described in Patent No. 2,205,854 to Kroll, and modifications thereof. Due to the presence of certain impurities, titanium of commercial purity as thus produced, possesses higher strength and greater hardness than that obtained by the Van Arkel or "iodide" process.

The present invention comprises in one of its aspects the discovery that strong and ductile binary alloys of titanium and aluminum are obtained over a critical range of about 2.5 to 8% aluminum.

The invention comprises in another of its aspects the further discovery that the strength of the binary alloy is greatly enhanced, without undue loss of ductility, by controlled additions of one or more of the interstitials carbon, oxygen and nitrogen. In the absence of appreciable amounts of oxygen and nitrogen in the alloy, the carbon may range up to about 0.6% on the high side with aluminum up to about 5% which additions as small as about 0.05% are effective materially to strengthen the binary alloy. Thus the addition of 0.05% carbon enhances the tensile strength by about 5,000 p. s. i. At higher aluminum contents, the maximum carbon must be proportionately reduced down to about 0.3% carbon at about 7.5% aluminum.

In the absence of appreciable amounts of carbon and nitrogen, oxygen may range up to 0.35% on the high side with aluminum up to about 5%; without undue embrittlement of the alloy, the lower effective limit being about 0.05%, with the same enhancement in tensile strength as is above indicated for the lower carbon limit. The oxygen content should be on the low side for aluminum contents upwards of 5%, i. e., above 5% aluminum; total oxygen should not exceed about 0.2%.

In the absence of appreciable amounts of carbon and oxygen, the nitrogen content may range up to 0.25% on

5

10

15

20

25

30

35

40

45

50

55

60

65

70

75

80

85

90

2

the high side for aluminum contents up to about 5%, without unduly embrittling the alloy, the lower effective limit being about 0.025%, with the same enhancement and strengthening effect as the lower limit additions of carbon and oxygen above noted. At upwards of 5% aluminum, total nitrogen should not exceed about 0.15%.

In the absence of any appreciable content of nitrogen, i. e., under about 0.025%, the carbon may range up to about 0.4%, together with oxygen up to about 0.2%, again with aluminum up to about 5%. Likewise, in the alloys containing both carbon and nitrogen, but inappreciable amounts of oxygen, the carbon may range up to about 0.25% in conjunction with nitrogen up to about 0.2%. Where all three elements, carbon, oxygen and nitrogen are present, the carbon should not exceed about 0.25%, and the total content of oxygen and nitrogen should not exceed about 0.2%. The alloys containing over 0.4% carbon are embrittled by additions of oxygen or nitrogen.

In the drawings, Fig. 1 is a series of curves showing the elongation and tensile properties of a series of binary "iodide" base titanium-aluminum alloys containing from 1 to 5% of aluminum.

Fig. 2 is a composite graph showing the elongation and 0.2% offset yield strengths of numerous "iodide" base titanium-aluminum alloys containing up to 8% of aluminum.

It has been found that the addition to titanium of 1 to 2% of aluminum has a relatively minor effect, the properties of the resulting alloys not differing materially from those of unalloyed titanium.

As shown in Fig. 1, alloys of titanium with 1% aluminum have, as compared with unalloyed titanium, an ultimate strength which is but slightly higher, and a yield strength and a proportional limit which are actually lower than those of the unalloyed metal. The change is elongation is slight.

A very significant change takes place in the region of an aluminum content of about 2.5%. The proportional limit and yield strength curves have actually reversed, both properties showing a defining increase. Ductility is diminished but is approaching a minimum value. As the aluminum content is further increased, say to 5%, the effect is even more striking. The second 2.5% increment produces an improvement in tensile properties which is several times that of the first 2.5% increment, but without a proportionate loss of ductility that would be expected. Instead, the loss of ductility is almost negligible, and substantially less than that taking place between a zero aluminum content and a 2.5% aluminum content.

The alloys of Fig. 1 were prepared and processed as follows:

An admixture of "iodide" titanium with the requisite amount of aluminum was melt cast under contamination-free conditions by arc melting in a cold mold or water-cooled crucible in an inert or argon atmosphere. The resulting ingot was heated to a temperature of about 850° C., and rolled to a thickness of about 0.040", its thickness being reduced about 10% at each pass through the rolls, and the ingot being reheated to about 850° C. after each pass. After being brought to the desired thickness, the strip was mechanically cleaned and vacuum annealed for about 3 hours at a temperature of about 850° C. The properties graphically illustrated in Fig. 1, together with those of a 7.5% aluminum alloy, are tabulated as follows:

Table I

(IODIDE TITANIUM BASE)

| Composition, Percent (Balance Titanium) | Vickers Hardness | Proportional Limit: | Yield Strength |             | Ultimate Strength | Elongation, 1" | Area Reduction |
|-----------------------------------------|------------------|---------------------|----------------|-------------|-------------------|----------------|----------------|
|                                         |                  |                     | 0.1% Offset    | 0.2% Offset |                   |                |                |
| 100Ti                                   | 103              | 7,000               | 23,200         | 27,100      | 30,900            | 29             | 66             |
| 1Al                                     | 138              | 6,200               | 21,000         | 24,800      | 44,100            | 28             | 66.5           |
| 2.5Al                                   | 193              | 8,800               | 30,100         | 33,800      | 52,200            | 20.5           | 54             |
| 5Al                                     | 270              | 43,000              | 60,800         | 63,100      | 78,900            | 17.5           | 43.5           |
| 7.5Al                                   | 320              | 90,100              | 91,100         | 91,300      | 96,500            | 22             | 35             |

Fig. 2 shows graphically the relationship between 0.2% offset yield strength and elongation for alloys of titanium with up to about 8% aluminum, being a composite of the results of numerous tests. Attention is particularly invited to the rapid increase in strength with slight loss of ductility when the aluminum content exceeds about 2.5%. These results are typical of many which the present applicants have secured for binary titanium-aluminum alloys subjected to a variety of processes, the titanium being either "iodide" or commercial purity titanium. For example, a series of alloys made with commercial purity titanium were subjected to the same processing as above outlined except that the final anneal at 850° C. was for a period of 15 minutes, instead of 3 hours, with the following results:

5 showed a Vickers hardness of 315; a proportional limit of 66,700; a 1% offset yield of 98,000, and a 0.2% offset yield of 103,500; an ultimate strength of 112,800; an elongation of 10; and an area reduction of 36.

These alloys are further characterized by their ability to maintain their hardness and strength at high temperatures. The hardness of an alloy of titanium with 5% aluminum materially exceeds that of 18-8 stainless steel 10 at all temperatures up to 600° C., and is equal to the hardness of such steel at about 700° C., and only slightly lower at 800° C. The binary alloys of this invention are thus of exceptional value for high temperature service, where they are preferred to the stainless steels by reason of their lighter weight.

Table II

| Composition,<br>Percent (Balance<br>Titanium) | Vickers<br>Hardness | Proportional<br>Limit | Yield Strength |                | Ultimate<br>Strength | Elonga-<br>tion, 1" | Area<br>Reduction |
|-----------------------------------------------|---------------------|-----------------------|----------------|----------------|----------------------|---------------------|-------------------|
|                                               |                     |                       | 0.1%<br>Offset | 0.2%<br>Offset |                      |                     |                   |
| 100Ti-----                                    | 210                 | 39,700                | 53,200         | 56,100         | 75,500               | 24                  | 3                 |
| 1Al-----                                      | 258                 | 41,000                | 59,100         | 63,000         | 77,700               | 23                  | 4                 |
| 2Al-----                                      | 258                 | 38,700                | 57,600         | 62,100         | 75,600               | 26                  | 4                 |
| 5Al-----                                      | 378                 | 102,000               | 114,000        | 115,000        | 121,000              | 16                  | 3                 |

Again the improvement, if any, due to the use of up to 2% aluminum is slight, while at 5% very high strength with ample ductility is found.

For alloys of slightly higher aluminum content a higher rolling temperature, say 1050° C., is preferred. For example, an alloy of "iodide" titanium with 8% aluminum, after rolling to a final thickness of 0.040" with a reduction of 10% per pass and a reheating to

The following Table III shows the effect on mechanical properties of additions of one or more of carbon, oxygen and nitrogen to the titanium-aluminum alloys of the invention. The results are given for both "iodide" base and commercial purity base titanium alloys as indicated in the table. Also the properties are for the alloys in the annealed condition, the specimens having been prepared by rolling and annealing at 850° C.

Table III.—Mechanical properties of Ti-Al and Ti-Al-(C, O, N) Alloys

[Annealed condition]  
(IODIDE TITANIUM BASE)

Table III.—Mechanical properties of Ti-Al and Ti-Al-(C, O, N) Alloys—Continued

[Annealed condition]  
(IODIDE TITANIUM BASE)

| Composition, Percent<br>(Balance Titanium) |      |     |       | Tensile Properties:<br>psi $\times 1,000$ |                      | Percent<br>Elongation<br>in 1" | Percent<br>Reduction<br>in Area | Vickers<br>Hardness | Min.<br>Bend<br>Radius<br>Long. |
|--------------------------------------------|------|-----|-------|-------------------------------------------|----------------------|--------------------------------|---------------------------------|---------------------|---------------------------------|
| Al                                         | C    | O   | N     | 0.2%<br>Offset<br>Yield                   | Ultimate<br>Strength |                                |                                 |                     |                                 |
| 5                                          | 0.25 | 0.2 | 0.925 | 141                                       | 143                  | 3                              | -----                           | 454                 | Brittle                         |
| 5                                          | 0.25 | 0.3 | 0.025 | -----                                     | 91                   | 0                              | 0                               | 481                 | Brittle                         |
| 5                                          | 0.25 | 0.2 | 0.05  | -----                                     | 103                  | 0                              | 0                               | 476                 | Brittle                         |
| 5                                          | 0.25 | 0.3 | 0.05  | -----                                     | 102                  | 0                              | 0                               | 473                 | Brittle                         |
| 5                                          | 0.25 | 0.2 | 0.075 | -----                                     | 137                  | 0                              | 0                               | 458                 | Brittle                         |
| 5                                          | 0.25 | 0.1 | 0.1   | 133                                       | 133                  | 1                              | 9                               | 443                 | Brittle                         |
| 5                                          | 0.25 | 0.2 | 0.1   | -----                                     | 82                   | 0                              | 0                               | 477                 | Brittle                         |
| 5                                          | 0.1  | --  | 0.1   | 106                                       | 116                  | 12                             | 25                              | 337                 | -----                           |

  

| (COMMERCIAL PURITY TITANIUM BASE) |      |      |     |     |     |    |    |     |       |
|-----------------------------------|------|------|-----|-----|-----|----|----|-----|-------|
| 4                                 | 0.1  | --   | --  | 99  | 105 | 17 | 49 | 324 | 1.7   |
| 4                                 | 0.2  | --   | --  | 108 | 113 | 19 | 52 | 345 | 1.8   |
| 5                                 | 0.1  | --   | --  | 126 | 133 | 15 | 31 | 402 | 5.0   |
| 5                                 | 0.2  | --   | --  | 122 | 131 | 22 | 43 | 404 | 2.4   |
| 5                                 | 0.25 | --   | --  | 137 | 143 | 18 | 37 | 427 | 5.5   |
| 4                                 | --   | 0.25 | --  | 107 | 115 | 17 | 46 | 355 | 2.6   |
| 4                                 | --   | 0.35 | --  | 119 | 127 | 13 | 29 | 380 | 2.7   |
| 5                                 | --   | 0.25 | --  | 109 | 118 | 17 | 37 | 405 | 3.1   |
| 5                                 | --   | 0.35 | --  | 123 | 132 | 19 | 33 | 411 | 3.5   |
| 4                                 | --   | --   | 0.1 | 110 | 117 | 17 | 42 | 350 | 1.8   |
| 5                                 | --   | --   | 0.1 | 130 | 137 | 14 | 38 | 398 | 2.5   |
| 5                                 | --   | --   | 0.1 | 106 | 116 | 12 | 25 | 337 | ----- |

<sup>1</sup> Includes 0.15% oxygen present in unalloyed titanium-base metal; the nitrogen and carbon contents were sufficiently small to be neglected.

From the above data it will be seen that the binary alloy containing up to about 5% aluminum is strengthened without undue loss of ductility by carbon additions of up to about 0.6%. Thus, whereas the "iodide" base Ti-5Al binary yield and ultimate strengths and tensile elongation values are, respectively, 63,000 p. s. i., 79,000 p. s. i. and 17.5%, in the Ti-5Al-0.6C ternary, these values become 122,000 p. s. i., 123,000 p. s. i. and 18%. Thus the yield strength has been doubled and the tensile strength increased by 50% with no loss of ductility.

At upwards of 5% aluminum the carbon content should be correspondingly reduced if adequate ductility is to be retained. Thus the "iodide" base Ti-7.5Al binary has an ultimate strength of 97,000 p. s. i. and a tensile elongation of 22% as compared to an ultimate of 125,000 p. s. i. and an elongation of 18% for the Ti-7.5Al-0.25C ternary alloy. Here again marked strengthening with no noticeable loss of ductility results from the carbon addition.

The ultimate strength of alloys of titanium with about 7.5% aluminum is increased by additions of carbon up to about 0.3%. These alloys have the peculiarity of sustaining a maximum load with an elongation less than 0.1%, then elongating about 20%, with an area reduction in excess of 40% before failure. They are rendered brittle by the presence of more than about 0.3% carbon, the 0.3% figure substantially coinciding with the solubility of carbon in alpha titanium. The alloys containing 5-7% aluminum with about 0.3% carbon, will not tolerate more than a few hundredths of one percent of either oxygen or nitrogen, being completely embrittled by 0.1% of either.

As further shown by the Table III data, for aluminum contents up to about 5%, the total oxygen content in the absence of appreciable amounts of carbon and nitrogen may range up to a total of about 0.35%. Here again, marked strengthening is obtained with no material effect on ductility. Comparing the values for the commercial purity titanium base alloys, the Ti-5Al binary has an ultimate of 121,000 p. s. i. and an elongation of 16%, as against an ultimate of 132,000 p. s. i. and an elongation of 19% for the Ti-5Al-0.35,O ternary. Above 5% aluminum, the total oxygen content should be held on the low side and not to exceed a total of about 0.2%.

For alloys containing up to 5% aluminum, the total nitrogen may range up to about 0.25% in the absence of appreciable amounts of carbon and oxygen, again with marked strengthening, although with considerable loss of ductility. Comparing the values for the "iodide" base Ti-5Al binary and the Ti-5Al-0.2N ternary, the ultimate strength is substantially doubled from 79,000 to 145,000 p. s. i. with accompanying reduction in tensile elongation from 17.5 to 2%. However, it will be observed that the bend ductility of the ternary is excellent, namely, 2.1 T. Above 5% aluminum the total nitrogen should not exceed about 0.15% in the ternary Ti-Al-N alloy.

The data further shows that these alloys containing up to 5% aluminum and up to 0.4% carbon, are further strengthened by additions of oxygen up to about 0.2%, although with considerable loss of ductility, the ultimate without and with the oxygen addition being 121,000 and 140,000, respectively, with corresponding elongations of 18% and 1%. Up to the 0.25% carbon level, however, considerable strengthening occurs with no loss of ductility; the comparisons for the ultimates and elongations are 108,000 versus 130,000 and 18% versus 19%, respectively, for the Ti-5Al and Ti-5Al-0.25C-0.2,O alloys. In the alloys of this group, the nitrogen content should not exceed 0.025%, as further shown by the Table III data. The data also shows that with carbon in excess of 0.4%, these alloys are embrittled by the presence of appreciable amounts of oxygen and/or nitrogen.

In the absence of significant amounts of oxygen, the alloys containing up to 5% aluminum and up to 0.25% carbon, are benefited by additions of nitrogen up to about 0.1% nitrogen, but become quite brittle for higher nitrogen additions. At the 0.1% nitrogen level the strength and ductility comparisons without and with this addition are 108,000 versus 122,000 p. s. i. for the tensiles and 18% versus 15% for the corresponding elongations. With this group of alloys the total oxygen and nitrogen should not exceed about 0.2%.

The alloys of the invention having tensile elongations as low as 1 or 2% are useful in forgings and those having a minimum bend radius as high as 20 T are useful in sheet form.

The alloys of the invention have excellent cold working properties as shown by the data on edge cracking

limits versus percent reduction given in the following Table IV:

Table IV.—*Cold working properties for Ti-Al and Ti-Al plus C, O, N alloys*  
(COMMERCIAL PURITY TITANIUM BASE)

| Composition, percent (Balance Titanium) | VHN (Annealed) | Cold Rolling Edge Cracking Limit, percent red. | VHN at 50% Reduction By Cold Rolling |
|-----------------------------------------|----------------|------------------------------------------------|--------------------------------------|
| 100Ti                                   | 104            | 183                                            | 289                                  |
| 1Al                                     | 237            | 77                                             | 325                                  |
| 2Al                                     | 295            | 67                                             | 330                                  |
| 4Al                                     | 307            | 35                                             | 2411                                 |
| 5Al                                     | 377            | 45                                             | 2397                                 |
| 8Al                                     | 389            | 25                                             | 2432                                 |

## (IODIDE TITANIUM BASE)

|                |     |     |      |
|----------------|-----|-----|------|
| 100Ti          | 106 | 186 | 208  |
| 1Al            | 132 | 185 | 232  |
| 2Al            | 153 | 183 | 251  |
| 3Al            | 212 | 181 | 283  |
| 4Al            | 244 | 71  | 282  |
| 5Al            | 273 | 68  | 318  |
| 6Al            | 317 | 47  | 320  |
| 6.5Al          | 307 | 29  | 316  |
| 7.5Al          | 320 | 31  | 353  |
| 5Al-0.25C      | 345 | 57  | 368  |
| 5Al-0.3C       | 335 | 63  | 367  |
| 5Al-0.4C       | 365 | 60  | 383  |
| 5Al-0.5C       | 365 | 57  | 390  |
| 5Al-0.25C-0.1O | 385 | 43  | 2407 |
| 5Al-0.25C-0.2O | 400 | 45  | 2443 |
| 5Al            | 287 | 50  | 291  |
| 5Al-0.1N       | 321 | 26  | 2447 |
| 5Al-0.16C      | 357 | 20  | 1377 |
| 5Al-0.11O      | 304 | 41  | 2345 |
| 5Al-0.1C       | 314 | 50  | 322  |
| 5Al-0.25C      | 337 | 50  | 346  |
| 5Al-0.6C       | 397 | 41  | 2354 |
| 5Al-0.1N       | 298 | 49  | 2331 |
| 5Al-0.2N       | 336 | 47  | 1352 |
| 5Al-0.1O       | 310 | 51  | 347  |
| 5Al-0.2O       | 338 | 45  | 2357 |

<sup>1</sup> Did not crack at maximum reduction shown.

<sup>2</sup> Hardness at maximum reduction in edge-cracking test.

Referring to the above data, it will be seen that the iodide titanium-base alloys containing up to 5% aluminum were cold reduced up to at least 70% before edge cracking occurred, and even at substantially the upper limit of 7.5% aluminum, reductions up to about 30% were obtained. For the commercial purity titanium-base binary alloys, the percent cold reduction up to the edge cracking limit was slightly lower for a given aluminum addition than for the iodide titanium-base alloys, although the reductions are roughly comparable within about 5% or so. Excellent cold reduction properties are also shown for the ternary and higher order alloys containing one or more of carbon, oxygen and nitrogen.

The effect of the cold working in increasing the hardness is shown by the Vickers hardness values (VHN) of each alloy in the annealed condition as compared to that after cold working. The work hardening response of these alloys is further illustrated by the yield strength values given in the following Table V:

Table V.—*Yield strengthens of cold-worked Ti-Al and Ti-Al plus C, O, N alloys*  
(COMMERCIAL PURITY TITANIUM BASE)

| Composition, Percent (Balance Titanium) | Yield Strength Annealed, 1,000 p. s. i. | Yield Strength, Cold Worked, <sup>1</sup> 1,000 p. s. i. |               |               |
|-----------------------------------------|-----------------------------------------|----------------------------------------------------------|---------------|---------------|
|                                         |                                         | 20% Reduction                                            | 40% Reduction | 50% Reduction |
| 100Ti                                   | 53                                      | 96                                                       | 107           | 112           |
| 2Al                                     | 67                                      | 104                                                      | 116           | 120           |
| 3Al                                     | 91                                      | 114                                                      | 123           | 127           |
| 5Al                                     | 96                                      | 126                                                      | 135           | 138           |
| 6Al                                     | 104                                     | 135                                                      | 143           | 147           |

## (IODIDE TITANIUM BASE)

|                |     |     |     |     |
|----------------|-----|-----|-----|-----|
| 5Al            | 66  | 87  | 91  | 93  |
| 5Al-0.25C      | 103 | 124 | 128 | 131 |
| 5Al-0.4C       | 121 | 140 | 146 | 150 |
| 5Al-0.25C-0.1O | 106 | 128 | 138 | 142 |

<sup>1</sup> Predicted from flow curves obtained during tensile tests of annealed material.

It will be seen that cold working markedly increases the strength of these alloys.

What is claimed is:

1. A titanium base alloy consisting essentially of about: 5 to 8% aluminum, up to 0.6% carbon, up to 0.35% oxygen and up to 0.25% nitrogen, said elements being present in such relative proportions, and said alloy being sufficiently free from other alloying elements tending to reduce ductility as to impart to said alloy a minimum tensile elongation of about 10% and an ultimate strength at least 30% in excess of that of the unalloyed titanium base metal.

2. A titanium base alloy consisting essentially of about: 2.5 to 8% aluminum, up to 0.6% carbon, up to 0.35% oxygen and up to 0.25% nitrogen, as produced by melting the alloying elements in such relative proportions and under conditions sufficiently free from other elements tending to reduce ductility, as to provide a resulting alloy having a minimum tensile elongation of about 10% and an ultimate strength at least 30% in excess of that of the unalloyed titanium base metal.

3. A titanium base alloy consisting essentially of about: 2.5 to 8% aluminum and at least one element selected from the group consisting of 0.05 to 0.6% carbon, 0.05 to 0.35% oxygen and 0.025 to 0.25% nitrogen, said elements being present in such relative proportions, and said alloy being sufficiently free from other alloying elements tending to reduce ductility as to impart to said alloy a minimum tensile elongation of about 10% and an ultimate strength of at least 100,000 p. s. i.

4. A titanium base alloy consisting essentially of about: 2.5 to 8% aluminum and at least one element selected from the group consisting of carbon, oxygen and nitrogen in minimum amount of 0.1% and in maximum amount of 0.6% for carbon, 0.3% for oxygen and 0.25% for nitrogen, said elements being present in such relative proportions and said alloy being sufficiently free from other alloying elements tending to reduce ductility as to impart to said alloy a minimum tensile elongation of about 10% and an ultimate strength of at least 100,000 p. s. i.

5. A titanium base alloy consisting essentially of about: 2.5 to 8% aluminum, 0.05 to 0.4% carbon and 0.05 to 0.2% oxygen, said elements being present in such relative proportions and said alloy being sufficiently free from other alloying elements tending to reduce ductility as to impart to said alloy a minimum tensile elongation of about 10% and an ultimate strength of at least 100,000 p. s. i.

6. A titanium base alloy consisting essentially of about: 2.5 to 8% aluminum, 0.05 to 0.25% carbon and 0.025 to 0.2% nitrogen, said elements being present in such relative proportions and said alloy being sufficiently free from other alloying elements tending to reduce ductility as to impart to said alloy a minimum tensile elongation of about 10% and an ultimate strength of at least 100,000 p. s. i.

7. A titanium base alloy consisting essentially of about: 2.5 to 8% aluminum, 0.05 to 0.25% carbon, 0.025 to 0.2% of at least one element of the group oxygen and nitrogen, said elements being present in such relative proportions and said alloy being sufficiently free from other alloying elements tending to reduce ductility as to impart to said alloy a minimum tensile elongation of about 10% and an ultimate strength of at least 100,000 p. s. i.

8. An alloy consisting of about: 2.5 to 8% aluminum, up to 0.6% carbon, up to 0.35% oxygen, up to 0.25% nitrogen, and the balance titanium, said elements being present in such relative proportions, and said alloy being sufficiently free from other alloying elements tending to reduce ductility as to impart to said alloy a minimum tensile elongation of about 10% and an ultimate strength at least 30% in excess of that of the unalloyed titanium base metal.

9. An alloy consisting of about: 2.5 to 8% aluminum, up to 0.6% carbon, up to 0.35% oxygen, up to 0.25% nitrogen, and the balance titanium, as produced by melting the alloying elements in such relative proportions and under conditions sufficiently free from other elements tending to reduce ductility, as to provide a resulting alloy having a minimum tensile elongation of about 10% and an ultimate strength at least 30% in excess of that of the unalloyed titanium base metal.

10. An alloy consisting of about: 2.5 to 8% aluminum, at least one element selected from the group consisting of 0.05 to 0.6% carbon, 0.05 to 0.35% oxygen and 0.025 to 0.25% nitrogen, balance titanium, said elements being

present in such relative proportions and said alloy being sufficiently free from other alloying elements tending to reduce ductility as to impart to said alloy a minimum tensile elongation of about 10% and an ultimate strength of at least 100,000 p. s. i.

11. An alloy consisting of about: 2.5 to 8% aluminum, at least one element selected from the group consisting of carbon, oxygen and nitrogen, in minimum amount of 0.1% and in maximum amount of 0.6% for carbon, 0.35% for oxygen and 0.25% for nitrogen, balance titanium, said elements being present in such relative proportions and said alloy being sufficiently free from other alloying elements tending to reduce ductility as to impart to said alloy a minimum tensile elongation of about 10% and an ultimate strength at least 30% in excess of that 15 of the unalloyed titanium base metal.

References Cited in the file of this patent

UNITED STATES PATENTS

|           |          |               |
|-----------|----------|---------------|
| 1,648,954 | Marden   | Nov. 15, 1927 |
| 2,370,289 | Chandler | Feb. 17, 1945 |
| 2,464,836 | Thomas   | Mar. 22, 1949 |

20

FOREIGN PATENTS

|         |         |               |
|---------|---------|---------------|
| 718,822 | Germany | Mar. 24, 1942 |
|---------|---------|---------------|

OTHER REFERENCES

5 Zeitschrift für Anorganische Chemie; Begründet von Gerhard Kruss (1910), Band 65, pp. 388 thru 393.

Mellor "Comprehensive Treatise on Inorganic and Theoretical Chemistry," vol. 7, page 10, published 1927.

Zeitschrift für Metallkunde, vol. 29 (1937), Kroll, pages 189-192.

International Correspondence Schools Textbook "Inorganic Chemistry," part II, page 26, first ed., Copyright 1944.

Metals Technology, February 1946, T. P. 1961, page 8.

Metal Progress, February 1949, page 195.

Metallurgia, April 1949, page 304.

Modern Metals, March 1950, page 37.